

149

Patented June 9, 1931

1,809,621

## UNITED STATES PATENT OFFICE

HARRY P. CORSON, OF LAKewood, OHIO, ASSIGNOR, BY MESNE ASSIGNMENTS, TO THE GRASSELLI CHEMICAL COMPANY, OF CLEVELAND, OHIO, A CORPORATION OF DELAWARE

## INHIBITOR

No Drawing.

Application filed August 9, 1928. Serial No. 298,630.

The present invention relates to inhibitors, such as tetramethyl—or tetraethyl thiuram sulfides. Their use for controlling the action of acids upon metals, and to processes of cleaning, pickling, scaling or removing oxides and other acid soluble deposits from metallic articles.

I have found that thiuram sulfides display the property of inhibiting the action of acids upon base metals, that is to say, acids containing small amounts of my novel inhibitors will not, or only to a slight degree, dissolve such metals with correspondingly lesser evolution of hydrogen.

Thiuram sulfides are chemical compounds of the general formula



in which R stands for hydrogen or a hydrocarbon radical and x for one of the numerals, 1, 2, 3, etc. They are easily produced from the corresponding dithiocarbamic acids or their salts.

The usual pickling and cleaning baths for metallic articles consist of dilute mineral acids such as sulfuric or hydrochloric acid. The articles are treated therewith at various temperatures and under conditions suited to the particular problem, it being understood that pickling of sheet steel or of steel stock for wires, for instance, may require different operations, concentrations of acid, temperature, etc., than scaling boiler tubes or freeing water pipes from rust and other acid soluble incrustations.

The addition of a small amount of a thiuram sulfide to the acids used in such operations will prevent or greatly reduce the attack of the acid on the metal itself, without materially affecting the dissolution of the scale, rust, and other incrustations. This results in a noticeable saving of acid, but the main advantage of the use of my novel inhibitors is the protection of the metal which is not weakened or pitted. Amounts of less than  $\frac{1}{2}$  of 1% of a thiuram sulfide figured on the weight of the bath is usually sufficient to produce the desired inhibiting effect. Amongst the various thiuram sulfides I found that some of the best inhibitors will be found amongst the tetra-alkyl derivatives

The beneficial effect of my novel inhibitors can easily be shown by measuring the gas evolved from a piece of metal immersed in a dilute acid.

The results tabulated below were obtained by measuring the gas evolved from test pieces of ordinary black mild sheet steel immersed for various periods of time at room temperature in 34% sulfuric acid. It will be noted that the inhibiting effect is inversely proportional to the amount of gas evolved:

| Composition of inhibitor         | Amount used<br>% of bath | Gas evolved in |       |       |       | 65       |
|----------------------------------|--------------------------|----------------|-------|-------|-------|----------|
|                                  |                          | c. c.          | 1     | 2     | 6     |          |
| No inhibitor used                |                          |                | Hours | Hours | Hours | Hours    |
| Thiuramdisulfide                 | 0.5                      | 55             | 33    | 210   | 1,010 | >2,000   |
| Tetramethyl-thiuram-mono sulfide | 0.1                      | 8              | 2     | 60    | 150   | >350     |
| Do                               | 0.5                      | 11             | 3     | 14    | 7     | 70       |
| Tetramethyl-thiuram - di sulfide | 0.1                      | 12             | 6     | 24    | 120   | REVERSED |
| Do                               | 0.5                      | 10             | 5     | 9     | 26    | 75       |

Mixtures of my various inhibitors or mixtures of these with other known inhibitors can be used and similar improved results obtained.

These inhibitors can also be used in the presence of the foam-producing agents commonly added to pickling baths without detriment to the effect of either.

It will be understood that my invention is not limited to the particular substances and procedures mentioned herein, but that it comprises the application of my novel inhibitors to the various operations carried out under various conditions involving the action of acid upon metal articles where it is desired to free the metal from acid soluble incrustations with least possible attack of the metal itself.

I claim:

1. A pickling and cleaning bath for metals comprising a dilute acid containing a small amount of a thiuram sulfide.
2. In a process for pickling and cleaning metal articles, the step comprising treating

said articles with a dilute acid containing a small amount of a thiuram sulfide.

3. A pickling and cleaning bath for metals comprising a dilute acid containing a small amount of a tetra-alkyl-thiuram sulfide.

5. A pickling and cleaning bath for metals comprising a dilute acid containing a small amount of a tetra-methyl-thiuram sulfide.

10. In a process for pickling and cleaning metal articles, the step comprising treating said articles with a dilute acid containing a small amount of a tetra-alkyl-thiuram sulfide.

15. In a process for pickling and cleaning metal articles, the step comprising treating said articles with a dilute acid containing a small amount of a tetra-methyl-thiuram sulfide.

20. The process of pickling metals which comprises subjecting the metal to a pickling solution which contains a thiuram sulphide.

25. The process of cleaning a metal surface which comprises treating such metal with a sulfuric acid solution containing a small proportion of a thiuram compound.

9. A pickling bath for iron and steel products comprising a pickle acid containing a dissolved thiuram compound.

In testimony whereof, I affix my signature.

HARRY P. CORSON.

30

158-7

(3)

### Certificate of Correction

Patent No. 1,809,621.

Granted June 9, 1931, to

HARRY P. CORSON

It is hereby certified that error appears in the printed specification of the above-numbered patent requiring correction as follows: Page 1, strike out the table between lines 65 and 75 and insert the following table instead:

| Composition of inhibitor                 | Amount used<br>% of<br>bath | c. c. gas evolved in |            |            |             |
|------------------------------------------|-----------------------------|----------------------|------------|------------|-------------|
|                                          |                             | 1<br>hour            | 2<br>hours | 6<br>hours | 20<br>hours |
| No inhibitor used.....                   |                             | 55                   | 210        | 1,010      | >2,000      |
| Thiuramdisulfide.....                    | 0.5                         | 33                   | 60         | 150        | >350        |
| Tetramethyl-thiuram-<br>monosulfide..... | 0.1                         | 8                    | 11         | 14         | 15          |
| Do.....                                  | 0.5                         | 2                    | 3          | 6          | 7           |
| Tetramethyl-thiuram-<br>disulfide.....   | 0.1                         | 10                   | 12         | 24         | 120         |
| Do.....                                  | 0.5                         | 5                    | 6          | 9          | 26          |

and that the said Letters Patent should be read with this correction therein that the same may conform to the record of the case in the Patent Office.

Signed and sealed this 25th day of August, A. D. 1931.

[SEAL.]

M. J. MOORE,  
Acting Commissioner of Patents.